

## UNITED STATES PATENT OFFICE.

REGINALD SCOTT DEAN, OF LA GRANGE, ILLINOIS, AND WILLIAM EWART HUDSON, OF LOS ANGELES, CALIFORNIA, ASSIGNEES TO WESTERN ELECTRIC COMPANY, INCORPORATED, OF NEW YORK, N. Y., A CORPORATION OF NEW YORK.

## STORAGE-BATTERY GRID.

No Drawing. Application filed February 5, 1924, Serial No. 690,720. Renewed September 27, 1927.

An object of this invention is to produce a storage battery grid of high lead content having greater hardness and tensile strength than has heretofore been possible 5 in such an alloy.

A further object of this invention is to produce a lead-alloy storage battery grid of low alloying content with increased tensile strength and hardness and maximum 10 resistance to corrosion.

Storage battery grids are usually made of lead, into which some alloying matter is added to increase the hardness and tensile strength of the lead. A common alloy employed consists of about 90 per cent lead 15 and 10 per cent antimony.

In our co-pending application, Serial No. 690,716, filed February 5, 1924, a method of greatly increasing the hardness and tensile strength of lead by adding a small amount of alloying matter and subjecting the alloy to a hardening treatment is disclosed. It is sufficient to state here that the process consists briefly in adding alloying 20 matter to lead which has a greater solubility at a higher temperature than at a lower temperature. A solid solution is formed at the higher temperature and the alloy quenched to a lower temperature, to 25 form a supersaturated solution, and subsequently allowed to age. A process for manufacturing storage battery grids according 30 to this method is as follows:—

The lead and antimony are prepared preferably in proportions of 97.75 per cent lead and 2.25 per cent antimony and cast into the form of an ingot and formed, therefrom into the shape of the grid desired. It is sometimes advantageous to roll the 35 ingot into a flat sheet and then stamp the grid of proper proportions therefrom. After the grid has been formed in this manner its alloy constituents are usually found to be in the form of a solid solution 40 of antimony in lead. If, however, the work performed on the alloy and the temperature maintained during the work have not been sufficient to cause the alloy to become a homogeneous solid solution, the grid must 45 be heated until a solid solution is formed. This formation of the solid solution may 50 be carried out in the manner set forth in detail in the co-pending application mentioned above. After the grid has been

formed and its alloy constituents reduced to 55 a solid solution it is quenched and aged. Quenching in water at room temperature has been found sufficiently efficacious, as such a temperature is low enough to accomplish the desired result, and is easily maintained. 60 Aging may take place at temperatures below about 100° C. but above about 0° C. For practical purposes, about 20° C. is sufficient. If aged at room temperatures, good results are found to be obtained in about 72 hours. 65

The preliminary steps in this process may be varied as follows:—

Lead and antimony preferably in the proportions of 97.75 per cent lead and 2.25 per cent antimony are melted together and 70 when in an entirely molten state are cast into the form required. When solid they are heated until a substantially homogeneous solid solution is formed, quenched and aged. Hardening may be obtained with percentages of antimony between about 1 per cent and 3 per cent but greatest hardness 75 is obtainable with about 2.25 per cent antimony.

A storage battery grid produced according to this method from an alloy of 97.75 per cent lead and 2.25 per cent antimony has a tensile strength of 12,000 pounds per square inch and a micro-Brinnell hardness of about 28. Unhardened alloy of 2.25 per cent antimony and 97.75 per cent lead has a hardness of 8, and a tensile strength of 80 about 4,000 pounds per square inch. Such a storage battery grid shows very much greater resistance to corrosion than is obtainable by alloying the lead to obtain 85 substantially the same properties of hardness and tensile strength.

It has been found that work performed on a lead alloy article during its fabrication has 90 the effect of diminishing the time required to reduce the alloy to a solid solution by heating. This fact can be made use of in the manufacturing of storage battery grids. For more specific details of a process for 95 hastening the formation of a solid solution by work during the progress of fabrication, reference may be made to our copending application No. 690,719, filed February 5, 1924.

By practicing the above outlined method, 100 storage battery grids may be produced which in their finished form consist of a lead alloy

in which the solute constituent is dispersed substantially uniformly throughout the lead in a very finely divided form. It is believed that the improved properties of such storage 5 battery grids result from the extreme smallness of the particles of the solute material and to the uniformity of their dispersion throughout the lead.

This invention is not confined to the use 10 of antimony as solute. Any alloying matter having the desired qualities as indicated in our copending application mentioned above may be used.

What is claimed is:

15 1. A storage battery grid formed of a lead alloy in which lead is the major constituent, characterized by the presence of finely divided particles of a solute material substantially uniformly dispersed throughout the lead.

20 2. A storage battery grid formed of a lead-antimony alloy in which lead is the

major constituent, characterized by the presence of finely divided particles of antimony substantially uniformly dispersed throughout the lead. 25

3. A storage battery grid formed of a lead-antimony alloy containing less than 3 per cent antimony, and characterized by the presence of finely divided particles of antimony substantially uniformly dispersed throughout the lead. 30

4. A storage battery grid formed of a lead-antimony alloy containing about 2.25 per cent antimony, and characterized by the presence of finely divided particles of antimony substantially uniformly dispersed throughout the lead. 35

In witness whereof, we hereunto subscribe our names this 22nd day of January A. D., 40 1924.

REGINALD SCOTT DEAN.  
WILLIAM EWART HUDSON.